

Aug. 24, 1926.

A. M. GRIMM

1,597,373

METHOD OF AND MOLD FOR MAKING PRESSED CEMENT TILES

Filed August 7, 1925



Witness:  
W. H. Hall

Alexander M. Grimm  
By Hazards and Miller  
Attorneys

## UNITED STATES PATENT OFFICE.

ALEXANDER M. GRIMM, OF HEMET, CALIFORNIA.

## METHOD OF AND MOLD FOR MAKING PRESSED CEMENT TILES.

Application filed August 7, 1925. Serial No. 48,735.

My invention is a method of and mold for making pressed cement tiles of variegated colors and pattern and in the molding blocks utilized therein and in the resulting product or tiles.

In the attempts to make molded cement tiles of variegated pattern and colors it has been difficult to obtain a true and distinct line between the different parts of the pattern and to prevent intermingling of the colors at their adjoining edge. Moreover, the variegated pattern which is usually a relatively thin face is often not secured to the back of the tile with a sufficient bond to form a permanent and in effect integral tile. In the prior procedure sometimes one or more of the colored sections of a tile become knocked away from the base thus spoiling the tile by insufficient bond therewith.

In the method of making my pressed cement tiles I utilize a smooth flat surface face plate which is preferably polished in order to effect a glaze on the tile as hereafter explained. The mold surrounding the rim of the plate is preferably made of steel in order to stand the high pressure of molding. In forming the mold I use a series of stencils or more properly called stencil blocks which are fitted in the mold to make the complete pattern of variegated tile. I prefer to use a full set of stencil blocks so that they may all be properly centered. These blocks are so constructed that they may be removed one at a time and the particular colored cement desired may be molded on the face plate before the other or adjacent tile stencil blocks are removed and the particular color cement inserted in their place.

In one method of procedure I provide the stencil blocks with curved edges so that in removing a block it may be rocked or pivoted on one side and withdrawn from position without disturbing the other blocks and likewise when the colored cement is molded in the place of the block the adjacent block can be tilted outwards with a curved motion without disturbing the surface edge of the freshly molded section. In some cases I also mold the different sections of the tiles of different depths so that they will have a

locking or bonding function at the back with the filling material of the tile.

My invention will be more readily understood from the following description and drawings, in which;

Figure 1 is a face view of a finished tile indicating one multicolored design.

Fig. 2 is a perspective view of the mold with the removable stencil blocks inserted therein prior to molding the face.

Fig. 3 is a cross section of Fig. 2 on a vertical plane on the line 3-3.

Fig. 4 is a section similar to Fig. 3 indicating the multicolored face sections molded with the backing material thereon and with the press block bearing on the backing material.

Fig. 5 is a section similar to Fig. 4 in which the face blocks of the stencil have been preferably all of the same level and the face sections of the tile are molded all of substantially the same thickness.

Referring to Fig. 1, which illustrates one form of a finished tile with a multicolored design, for purposes of illustration the different portions are illustrated with a simple design in which the central section 1 is indicated as being a black color, the adjacent section 2 a red and the small lateral sections 3 as a yellow color. These face sections are molded to a tile backing material as hereafter described.

Referring particularly to Figs. 2 and 3, the molding face plate 4 is preferably made of steel with a polished face and the mold 5 is preferably formed of a heavy strong metal to withstand the pressure of molding as hereafter described. The stencil blocks are designated generally by the numeral 6 in which the central block 7 forms the mold for the black color 1, the angular stencil blocks 8 for the red color 2 and the outer segmental blocks 9 for the yellow color 3. These blocks are preferably provided with a screw threaded recess 10 in which is inserted a removable stem 11. These stems may however, be permanently attached to each mold section but for intricate work it is desirable to remove the stems so that the individual colored sections of cement may be properly molded into position.

As shown in Fig. 3, the various blocks are formed with a bevelled edge 12 where they abut each other. The central block 7 is shown with a straight bevel whereas the outer edge of the angular block 8 is shown with a curved edge 13 formed on a radius from the point 14 where its upper edge 15 contacts with the edge of the central block 7. The outside segmental blocks 9 are also formed with a curved edge 16 where they contract with the mold 5, the radius of the curve being drawn from the point 17 where the upper edge contacts with the outer edge of the adjacent blocks 8.

15 As illustrated in Figs. 2 and 3 the various stencil blocks are of different thicknesses but if desired they may also be made of a uniform thickness and the bevelled and curved edges may be reversed so that the inner section will be the first to be removed instead as shown being the last to be removed.

The operation of molding the colors is substantially as follows:—As above described I prefer to fill the mold completely with 25 the stencil blocks so as to center the pattern properly and uniformly for each tile to be molded. In the design shown the outer segments 9 are removed by pivoting them upwardly using the point 17 as a center of 30 rotation. The cutaway portion or as it may be termed the under cut edge formed by the curve 16 allows this section to be removed although its upper outside edge is in close engagement with the inner face of 35 the mold.

The colored cement in this case indicated as yellow, after being properly dampened preferably with a soapy water, is sprinkled on to the face plate 4 in each section where 40 the stencil blocks 9 have been removed. This colored cement is then slightly molded until it is pressed into the outside under cut part of the adjacent mold block 9 formed by the curve 13 and is molded against the mold 45 5 to give clear distinct and sharp edges. This may be spread to the desired thickness and may be as thin as one-eighth of an inch.

The next adjacent stencil blocks 8 are then removed by carefully pivoting them upward 50 as if rotated on the center 14 so that the outer curved edge 13 will draw clear of the outer molded section without disturbing the edge against the face plate 4. A colored cement indicated as a red and prepared as 55 above described is then molded into the space vacated by the stencil blocks and as indicated by Fig. 4 this color is molded slightly thicker than the outside color.

The inner block 7 is then removed, and as 60 illustrated on account of the bevels 12, may be lifted vertically. The central color is then sprinkled and molded into the space vacated by these blocks, being if desired slightly thicker than the adjacent sections.

65 The mold is then filled to the desired depth

to give the thickness of tile required with a suitable cement properly moistened and mixed with sand, using either an ordinary quick or a slow setting cement. The press block 20 is then inserted on top of the filling 70 21 and subjected to a high pressure such as about 1000 pounds per square inch. The higher the pressure the more glassy is the surface of the finished tile.

The tiles are then removed from the mold 75 by separating the face plate 4, the mold 5 and the press block 20 and are preferably allowed to stand for twenty-four hours exposed to the air and are then submerged in water for varying lengths of time from a few minutes to a day or more according to the cement used. After submergence they are dried and the surface polished to a desired extent.

In some classes of more or less rough 85 work the edges of the stencil blocks may be made vertical, that is at right angles to the face plate 4 instead of being formed on bevels and curves as illustrated in Fig. 3 and 90 would thus form molded sections of the different colors with substantially a vertical line separating each section as indicated in Fig. 5. These sections may also be molded to a uniform height if desired and to do so the stencil blocks would preferably all be 95 the same height.

It is to be noted that in the procedure of 100 molding as described in connection with Figs. 3 and 4 the different sections in being molded slightly higher than the adjacent 105 sections, can be spread out to form a species of dove tailed edges 23 which will more firmly interlock and bond with the backing material. Moreover, the sections being of different height, even if not molded outwardly, give a better bonding than the sections all of the same thickness.

By this procedure, if I am making floor 110 tiles I can use a softer material for the deeper sections which will not form as hard a wearing surface as for the others and by the rubbing action or by use on a floor these tiles acquire the appearance of antique tiles as used several centuries ago.

It will be obvious that the designs of tiles 115 may be varied almost without limit and that the procedure may be reversed in forming the central portion of the tile first and then working towards the outside. Also in more or less rough work it is not necessary to complete the filling of the mold with the stencil blocks before molding the cement. Other modifications of my invention may be developed to suit special requirements 120 without departing from the spirit of my invention.

Having described my invention, what I claim is:

1. The method of making substantially 125 flat cement tiles face down, comprising 130

- building up a design with stencil blocks face down in a mold, said blocks fitting close together with substantially no vacant space therebetween, removing certain of the blocks 5 upwardly, filling the space vacated thereby with a cement inserted downwardly, removing other blocks upwardly, filling the space so formed with other cements inserted downwardly and allowing the cements to set 10 into a unitary tile.
2. The method of making substantially flat cement tiles face down, comprising forming a pattern with stencil blocks in a mold face down, said blocks fitting close together with substantially no vacant space 15 therebetween, removing certain of the stencil blocks upwardly, molding and pressing cement inserted downwardly into the space vacated, removing an adjacent block upwardly, molding cement inserted downwardly into the space vacated, said cement binding on the first mold of cement, removing a third block upwardly and molding a cement inserted downwardly into the space 20 vacated and allowing the different sections of cement to set forming a unitary tile.
3. The method of forming a substantially flat faced pressed cement tile comprising forming a complete pattern with stencil 25 blocks in a mold face down, removing upwardly different stencil blocks indicating different features of the design in succession and as each is removed molding a cement downwardly, the cement being of different 30 colors or characteristics in the place vacated by the blocks, molding the different sections of different depths, placing a backing material in the mold and pressing the backing material to form a unitary tile.
4. The method of forming a pressed cement tile as claimed in claim 3, comprising removing certain of the blocks in a curved direction and pressing the cement of the different sections partially under a projecting 45 part of the different blocks.
5. A mold for making cement tiles comprising in combination a flat base plate, a mold wall extending upwardly around the base plate and a series of independent stencil blocks inserted in the mold resting on 50 the base plate, forming a complete pattern, said blocks fitting close together, leaving substantially no vacant space.
6. A mold for making cement tiles as claimed in claim 5, in which some of the 55 blocks are thicker than others and adapted to form a guide for leveling off molded cement when an adjacent block is removed.
7. A mold for making cement tiles as claimed in claim 5, in which some of the 60 blocks are formed of curved edges to allow said blocks to swivel against adjacent blocks with a hinging motion.
8. A mold for making cement tiles, comprising in combination a face plate, a mold 65 surrounding the plate and extending upwardly therefrom, a series of independent stencils in the mold forming a complete design, some of said sections having convex and concave adjoining edges, such edges 70 being formed on a radius substantially equal to the width of the tile having the convex edge.
9. A stencil block for forming cement blocks of variegated sections, having a flat 75 lower face, a convex edge on one side, said convex edge forming a substantially undercut part of a block against which cement may be molded and said convex edge being substantially of the same radius as the distance from the lower undercut edge to the upper opposite edge, to allow removal of the block from a molded section of the tile with a curved motion.
10. The method of forming a substantially flat faced pressed cement tile, comprising forming a complete pattern with stencil blocks in a mold face down, removing upwardly different stencil blocks indicating 80 different features of the design in succession and as each is removed molding a cement downwardly, the cement being of different colors or characteristics in the place vacated by the blocks, molding the different sections of different depths, and placing a 85 backing material in the mold.

In testimony whereof I have signed my name to this specification.

ALEXANDER M. GRIMM.